

Sept. 18, 1923.

1,468,362

M. L. HARTMANN

SAFE OR VAULT PLATE

Filed April 25, 1922

*Fig. 1.*



*Fig. 2.*



INVENTOR

Miner L. Hartmann

by Byrnes, Stubbins, Angus & Hartmann  
his Attorneys

Patented Sept. 18, 1923.

## UNITED STATES PATENT OFFICE.

MINER L. HARTMANN, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## SAFE OR VAULT PLATE.

Application filed April 25, 1922. Serial No. 556,434.

*To all whom it may concern:*

Be it known that I, MINER L. HARTMANN, a citizen of the United States, residing at Niagara Falls, in the county of Niagara and State of New York, have invented a new and useful Improvement in Safe or Vault Plates, of which the following is a full, clear, and exact description, reference being had to the accompanying drawings, forming part of this specification, in which—

Figure 1 is a plan view of a safe or vault plate made in accordance with my invention, and

Figure 2 is a cross section of the same.

The object of my invention is to provide plates for vaults or safe walls which are more or less impregnable to the action of high temperature agents and flames, such as the oxy-acetylene flame.

As safes and vaults have heretofore been constructed it is possible by means of the oxy-acetylene flame to cut or burn holes through the walls or doors and gain access to the interior compartment.

My invention consists in embedding in a matrix of cast metal more or less closely assembled fragments of a highly refractory material which is not only infusible or difficultly fusible at the temperature reached by the oxy-acetylene flame but is also not acted upon by the highly heated and fluid iron oxide nor by oxygen. The material which I employ for the above purpose is fused ore of chromium oxide, preferably fused chromite. This material has a melting point which varies from about 1800° C. to about 2000° C. depending upon its purity.

The material may be made in accordance with the method set forth in my application Serial No. 556,426, filed April 25, 1922, that is to say, the ore of chromium oxide is subjected to high temperature and is fused in a non-reducing environment. This may be accomplished in any ordinary form of arc furnace with vertical electrodes depending into the furnace pot. The electrodes may

be of carbon or graphite. Graphite is preferred on account of the lessened amount of reduction which takes place from the carbon of the electrode. The furnace pot is preferably lined with refractory material such as chrome brick. The ore is fed into the furnace around the electrodes and a mass of fused chromite forms under the action of the arc. This material accumulates and builds up and spreads out in a fused condition for some distance outside of the arc. The electrodes are then raised to allow the mass to cool whereupon it solidifies into a pig or ingot of considerable size.

In the drawings, 2 represents the cast metal of the plate and 3 the fragments of fused chromium ore or chromite embedded therein.

In making a slab or plate for use in the construction of a burglar proof vault I prepare a dry sand mold of the required shape and of a character such as is used in the making of steel castings. In this I place fragments of fused chromium ore or chromite and then pour the molten metal, such as iron or steel into the mold in the usual manner. In a slab 10 inches thick, for instance, I would use fragments from 2 inches to 5 inches in diameter. The molten metal should be in a highly heated and very fluid condition so that it will flow around and penetrate all of the interstices of the mass of fragments and form a strong, tough, close, dense matrix therefor. If preferred the fragments may be preheated so as not to chill the metal. Any metal or alloy may be used as a matrix. The fragments may fill the entire mold and extend into every part of the slab or plate or they may be disposed in the center of the slab or otherwise disposed without departing from the spirit of my invention.

By the word "metal" in my claims, I intend to cover either substantially pure metals or alloys.

The invention is not limited to its preferred embodiment, the details of which

have been above set forth, but may be otherwise embodied within the scope of the following claims.

I claim:

- 5 1. As a new article of manufacture, a safe or vault plate formed of cast metal having embedded therein fragments of fused chromite in a dense compact mass.
2. As a new article of manufacture, a safe or vault plate formed of cast metal having

embedded therein fragments of fused ore of chromium oxide.

3. As a new article of manufacture, a safe or vault plate formed of cast metal having embedded therein fragments of fused chromite in a dense compact mass.

15 In testimony whereof I have hereunto set my hand.

MINER L. HARTMANN.